

# United States Patent Office

3,119,776

Patented Jan. 28, 1964

1

3,119,776

## LUBRICANT COMPOSITION

John R. Thomas, Lafayette, and Louis de Vries, Kentfield, Calif., assignors to California Research Corporation, San Francisco, Calif., a corporation of Delaware  
No Drawing. Filed Sept. 6, 1960, Ser. No. 53,908  
4 Claims. (Cl. 252—51.5)

This invention relates to a superior new lubricant composition. More particularly, the invention is concerned with a novel polymer thickened lubricant composition having an improved viscosity index and a remarkable resistance to shear degradation.

Constant effort is being made to produce lubricants which exhibit relatively little change in viscosity over a wide range of temperatures. Thus, in any application where a lubricant is subject to use in wide variations of temperature, it is desirable that the lubricant have not too high a viscosity at the lower temperatures, nor too low a viscosity at the higher temperatures. For effective lubrication the oil must not become so viscous at the lower temperatures so as to impede starting and cause excessive wear, and not become so thin at the higher temperatures so as to fail to provide adequate separation of the wearing surface.

With regard to lubricating oils, these desired viscosity-temperature characteristics may be obtained in some measure by the incorporation of certain synthetic products of large molecular size and comparative chemical inertness. These products are known as viscosity index (V.I.) improvers. However, any initial rise in V.I. attributable to the incorporation of the high molecular weight product will diminish upon operation of the machinery due to the shear forces set up by the moving parts of the machinery, for example, as in an internal combustion engine. These forces serve to shear the high molecular weight additive into component parts of lower molecular weight, yielding in turn a lower V.I. It can thus readily be seen that a high resistance to shear degradation is an exceptionally desirable property of a lubricant composition. A further highly desirable property of a lubricant additive composition is that a desired improvement in V.I. can be achieved by the addition to the lubricating oil of a small percent by weight of the additive.

It has now been found that lubricant compositions consisting of a major proportion of an oil of lubricating viscosity and a minor proportion, sufficient to improve the viscosity index of said oil, of a novel class of oil-soluble high molecular weight polypeptides derived from esters of optically-active glutamic acid exhibit remarkably each of the above described highly desirable properties. These novel polypeptides provide surprisingly effective lubricant thickening at low concentrations. Further, these novel polypeptides display a highly remarkable resistance to permanent shear degradation. This unusual combination of effective thickening power, low percent by weight additive requirement, and excellent shear strength, makes these novel polypeptides particularly desirable and useful as V.I. improvers.

The polypeptides of the present invention have the following general formula:



where R is selected from the group consisting of benzyl radicals, and alkyl radicals containing from 8 to 18 carbon atoms. The benzyl radical will occupy from 0 to 30 mol. percent of the ester radical (R) positions and the alkyl radical will occupy from 70 to 100 mol. percent of the ester radical positions. The molecular weight of the polymer will range from 10,000 to 1,000,000 with "n"

2

being the number of recurring units necessarily corresponding to the molecular weight.

These polyesters may be suitably prepared by transesterification of polybenzyl glutamate with the appropriate alcohol, or by direct synthesis from the glutamate monomer. The following specific examples will serve to illustrate the preparation of the products of the present invention, in particular, polylauryl glutamate.

## EXAMPLE I

10 Trans-esterification of polybenzyl glutamate: A 14.49 g. quantity of poly- $\gamma$ -benzyl-L-glutamate is dissolved in 250 cc. of dry chloroform. 170 cc. of dry lauryl alcohol is added with stirring and heating, along with 20 cc. of a mixture made from 7.86 g. of p-toluenesulfonic acid monohydrate and 600 cc. of benzene, wherein all water was removed by azeotroping. The mixture is refluxed for 48 hours, thereafter the solution is kept at 100° C. for six hours. At the end of this time no polymer should precipitate upon the addition of isoctane. The polymer is now precipitated by pouring the solution into excess methanol and filtering. The product is a white, fibrous polymer having a composition corresponding to 87% polylauryl glutamate and 13% polybenzyl glutamate, and having an estimated average molecular weight of about 150,000 as determined by viscosity measurements.

## EXAMPLE II

30 Direct synthesis from the glutamate monomer: 145 g. of glutamic acid is suspended in a mixture of 1 liter of dry distilled lauryl alcohol and 1 liter of sodium dried dioxane. 2.50 ml. of concentrated HCl (36%) is added and the mixture heated at 70° C. with stirring until the glutamic acid is dissolved. The solution is cooled to room 35 temperature and diluted with 2 volumes of ether. After three hours, the crystallization of lauryl glutamate hydrochloride is complete. The crystals are filtered and washed with pentane. Yield, 43.5 g. of the hydrochloride as shimmering flakes. Then the anhydride is prepared by 40 suspending 60 g. of the hydrochloride in dry chloroform and bubbling phosgene through the refluxing solution with vigorous stirring until a clear solution is obtained (approx. six hours). After vacuum removal of the excess phosgene and solvent the residue is diluted with a dry n-heptane and the solution cooled to 0° C. Crystallization, initiated by scratching, is complete after 12 hours. After filtration the solution is recrystallized at -30° C., 45 collected and dried. Yield, 25 g. of the anhydride as colorless flakes. Polymerization is accomplished by dissolving 5 g. of the anhydride in 100 cc. of dry benzene and adding 0.1 cc. of a solution of 36 mg./cc. of triethylamine in dry benzene. After standing for 40 hours, the viscous solution is poured into methanol and the precipitated polymer collected by filtration. The poly-50 lauryl glutamate product is a white, fibrous solid somewhat sticky to the touch. Yield, 95% completion of the reaction based upon the anhydride.

|                 | C     | H     | N    |
|-----------------|-------|-------|------|
| Calculated..... | 68.63 | 10.51 | 4.70 |
| Found.....      | 68.53 | 10.38 | 4.92 |

65 In general, excellent viscosity indexes can be imparted to lubricating oils by dissolving in them a quantity of from about 0.1 to 10% by weight of the polymers of the type described above, although a preferred range is from about 0.1 to 3% by weight. On the other hand, since the polymers of this invention are compatible with mineral and other lubricating oils in substantially all proportions, as much as 75% of the present polymeric additives can be dissolved in a suitable lubricating oil for the

purpose of preparing a concentrate capable of dilution with lubricating oils and the like to prepare the final lubricant composition. Such concentrates, which may also contain other additives in desired amounts, and which normally contain at least 10% of the polymer, comprise a convenient method for handling the polymer and may be used as a compounding agent for lubricants in general.

The polymeric additives of this invention can be used with good effect in the case of any one of a wide variety of oils of lubricating viscosity, or of blends of such oils. Thus, the base oil can be a refined Pennsylvania or other paraffin base oil, a refined naphthenic base oil, or a synthetic hydrocarbon or nonhydrocarbon oil of lubricating viscosity. As synthetic oils there can be alkylated waxes and similar alkylated hydrocarbons of relatively high molecular weight, hydrogenated polymers of hydrocarbons, and the condensation products of chlorinated alkyl hydrocarbons with aryl compounds. Other suitable oils are those which are obtained by polymerization of lower molecular weight alkylene oxides such as propylene and/or ethylene oxide. Still other synthetic oils are obtained by etherification and/or esterification of the hydroxy groups in alkylene oxide polymers such as, for example, the acetate of the 2-ethylhexanol-initiated polymer of propylene oxide. Other important classes of synthetic oils include the various esters as, for example, di-(2-ethylhexyl) sebacate, tricresyl phosphate, and silicate esters such as hexa (2-ethyl butoxy) disiloxane. If desired, the oil can be a mixture of mineral and synthetic oils.

While satisfactory lubricant compositions can be obtained by adding to the base oil employed only one or more of the polymeric additives of the type described above, it also falls within the purview of this invention to provide lubricant compositions which contain not only such polymers, but also other additives such as oiliness and extreme pressure agents, anti-oxidants, corrosion inhibiting agents, blooming agents, the temperature-viscosity characteristics of the oil. The present invention also contemplates the addition to the lubricant composition (particularly when the amount of copolymer employed is relatively small) of detergents and/or anti-wear agents.

Illustrative lubricant compositions of the above type containing the polymeric additives of the invention in combination with other agents may include, for example, from about 0.1 to 10% by weight of alkaline earth metal higher alkylphenate and sulfonate detergents, such as calcium alkylphenates having an average of approximately 14 carbon atoms in the alkyl group and basic calcium petroleum sulfonate, as well as organic thiophosphate corrosion and high temperature oxidation inhibitors such as the reaction product of pinene and  $P_2S_5$  and the bivalent metal dihydrocarbyl dithiophosphates, zinc butyl hexyl dithiophosphate and zinc tetradecylphenyl dithiophosphate in amounts of from about 0.1 to 10% by weight of the composition.

The superior properties of these novel lubricant compositions are illustrated by data compiled in the following tables.

In Table I various amounts of polyglutamate are incorporated in solvent-refined 150 neutral mineral lubricating oil in terms of percent by weight, and the improvement in viscosity and the surprising resistance to shear degradation corresponding to the low percent by weight polyglutamate additive is observed. The V.I. is determined by ASTM Standard Method D-567-41. The shear loss is determined by applying shear forces in the form of cavitations induced by ultrasonic waves and measuring the change in viscosity at 210° F. before and after cavitation. The polyglutamate employed is the trans-esterification reaction product of poly- $\gamma$ -benzyl-L-glutamate and lauryl alcohol, having a composition corresponding to approximately 90% polylauryl glutamate and 10% polybenzyl glutamate. Samples Numbers 1 through 5 have an average molecular weight of about 75.

500,000 and sample Number 6 has an average molecular weight of about 160,000.

Table I

## OIL-POLYGLUTAMATE SOLUTION PROPERTIES

| Sample No. | Percent by Weight Polyglutamate in 150 N Oil | Viscosity Sayboldt Seconds Universal at 210° F. | Viscosity Index | Percent Shear Loss (Δ Viscosity at 210° F.) |
|------------|----------------------------------------------|-------------------------------------------------|-----------------|---------------------------------------------|
| 10         | 0.0                                          | 42.2                                            | 87              | -----                                       |
|            | 0.085                                        | 79.9                                            | -----           | -----                                       |
|            | 0.13                                         | 59.6                                            | 120             | 42.8                                        |
|            | 0.18                                         | 59.6                                            | 119             | 56.3                                        |
|            | 0.26                                         | 52.5                                            | -----           | 10.9                                        |
|            | 0.5                                          | 67.2                                            | 120             | 2.8                                         |

Table II illustrates the superior thickening power of the above described polyglutamate as compared to commercially acceptable V.I. improvers. Acryloid 763 is a polymethacrylate V.I. improver having an average molecular weight of about 400,000, sold by Rohm & Haas. Paratone N is a polybutylene V.I. improver having an average molecular weight of about 120,000, sold by Enjay Co. The amount of additive that must be incorporated in 150 N oil to raise the viscosity of the oil at 210° F. to 67.2 SSU is measured and compared.

Table II

## COMPARATIVE THICKENING POWERS

|                                                                       | Polyglutamate | Acryloid 763 | Paratone N |
|-----------------------------------------------------------------------|---------------|--------------|------------|
| Weight percent additive required to yield oil of equal viscosity----- | 0.5           | 3.05         | 3.0        |

Table III illustrates the superior shear performance of the present invention as compared to the above mentioned commercial additives. The shear loss is determined by the method described above. The oil tested is at an additive concentration that will yield an oil of 67.2 viscosity, SSU at 210° F.

Table III

## COMPARATIVE SHEAR STRENGTH

|                                               | Polyglutamate | Acryloid 763 | Paratone N |
|-----------------------------------------------|---------------|--------------|------------|
| Percent Shear Loss (Δ Viscosity 210° F.)----- | 2.8           | 30.0         | 6.0        |

From the tests in Table I, it will be seen that each of the illustrative compositions containing the polyglutamate thickener possess remarkably improved viscosity-temperature properties compared to the base oil alone. Further, this improvement in viscosity-temperature behavior is achieved with the incorporation of a surprisingly small percent by weight of the polyglutamate, as is illustrated by Table II above. By comparison, commercially acceptable V.I. improvers such as the Acryloids or Paratones are normally employed in the amount of 1 to 5% by weight of the lubricating oil solution, whereas, approximately  $\frac{1}{10}$  of a percent by weight of the present invention provides sufficient thickening. Specifically, to raise the viscosity of 150 neutral oil to 67.2 SSU at 210° F. 6 times more Acryloid 763 or Paratone N is required than is required of the polyglutamate thickener, see Table II.

Similarly, it can be seen from Table III that, for an oil-additive solution of a viscosity of 67.2 SSU at 210° F. the present invention displays a 2.1 times greater shear strength than Paratone N and a 10.6 times greater shear strength than Acryloid 763.

We claim:

1. A lubricant composition comprising a major portion of an oil of lubricating viscosity and a minor

## 5

proportion, sufficient to improve the viscosity index of said oil of poly-gamma-esters of optically active glutamic acid having recurring units of the following formula



wherein said gamma ester R radicals are selected from the group consisting of 0 to 30 mol. percent benzyl radicals and from 70 to 100 mol. percent of alkyl radicals containing from 8 to 18 carbon atoms, the molecular weight of said polyester ranging from 10,000 to 1,000,000 and  $n$  being the number of recurring units corresponding to said molecular weight.

2. A lubricant composition comprising a major proportion of an oil of lubricating viscosity and a minor proportion, sufficient to improve the viscosity index of said oil of the poly-gamma-esters of optically active glutamic acid having recurring units of the following formula



wherein said gamma ester R radical is selected from the group consisting of 0 to 30 mol. percent benzyl radicals and from 70 to 100 mol. percent of the lauryl radical, the polyester having a molecular weight of 10,000 to 1,000,000 and  $n$  being the number of recurring units corresponding to said molecular weight.

3. A lubricant composition comprising a major proportion of an oil of lubricating viscosity and a minor proportion, sufficient to improve the viscosity index of said

## 10

oil of the poly-gamma-esters of optically active glutamic acid having recurring units of the following formula

5



wherein said gamma ester R radical is selected from the group consisting of 0 to 30 mol. percent benzyl radicals and from 70 to 100 mol. percent of the n-octyl radical, the polyester having a molecular weight of 10,000 to 1,000,000 and  $n$  being the number of recurring units corresponding to said molecular weight.

4. A lubricant composition comprising a major proportion of an oil of lubricating viscosity and a minor proportion, sufficient to improve the viscosity index of said oil of the poly-gamma-esters of optically active glutamic acid having recurring units of the following formula

20



wherein said gamma ester R radical is selected from the group consisting of 0 to 30 mol. percent benzyl radicals and from 70 to 100 mol. percent of the tridecyl radical, the polyester having a molecular weight of 10,000 to 1,000,000 and  $n$  being the number of recurring units corresponding to said molecular weight.

30

## References Cited in the file of this patent

## UNITED STATES PATENTS

2,368,604 White ----- Jan. 30, 1945  
 2,752,312 Dixon ----- June 26, 1956